

Sept. 20, 1927.

E. E. CHANDLER

1,643,198

METHOD OF COTTON STAPLING

Filed May 7, 1925



Fig 1



Fig 2

*Elbert E. Chandler*

INVENTOR.

## UNITED STATES PATENT OFFICE.

ELBERT E. CHANDLER, OF LOS ANGELES, CALIFORNIA.

## METHOD OF COTTON STAPLING.

Application filed May 7, 1925. Serial No. 28,696.

My invention relates particularly to cotton fibers, although it may well be applied to other fibers or bodies of varying lengths. Estimation of the length of cotton fiber is called stapling. Since the lengths of the fibers of any particular sample of cotton vary greatly, the art of stapling is rather difficult to acquire and considerable differences of opinions occur among experts as to the proper length to assign to any sample. The stapler takes a bunch of cotton in his two hands and pulls it into two portions. He discards one and from the other with his free hand he draws and laps successive pulls of fiber, by grasping the projecting ends between his thumb and fore finger. These pulls are laid over each other as evenly as possible and the process repeated. Projecting fibers are then drawn from the bundle and discarded. The bundle then assumes more or less the shape of a rectangular parallelogram. It is then laid on some surface and its length estimated. The stapler may also draw a line across each end and measure between the lines with a rule. He may even gain a pretty good idea of the length of the cotton when he pulls the first bunch into two parts, by noting the resistance to its being drawn apart. The more the bundle is evened up the shorter it becomes as the longer fibers naturally project and are rejected. It is difficult to determine where to draw the lines between which to measure. The length assigned in this process is frequently called the "body length" and is known to be considerably above the average length of the fiber.

This method is suitable to commercial operations, because of its rapidity, but greater accuracy is desirable for spinning and standardization purposes. Due to climatic and cultural conditions as well as to variety of the plant, cotton differs greatly in staple value not only in the bale, but also in the boll and even on the seed. Cotton of apparently the same body length may differ very much in average length as the device known as the Baer sorter readily shows. Because of physical and psychological differences estimates by different staplers often differ by one eighth of an inch although careful work may reduce the error to one sixteenth of an inch. Since large premiums are paid for extra lengths and in order to standardize the cotton standards as well as

the standardizers, the present method was developed.

This method consists of cutting a certain length from the middle portion of one or more bundles, tufts or pulls of cotton, combining the ends into one mass and the middles into another and determining the ratio of the ends to the middle by weight. 60

The device for doing the cutting is illustrated in Figures 1 and 2. It consists of a straight edge 1 of Figure 1, hinged at one end to the block 2 and clampable at the other to the block by means of the wing nut 3 and bolt attached to the block. The straight edge is slotted so that the bolt can be swung 65 out on a slight loosening of the nut. A zinc or brass plate 4 is placed between the edge and the block and the cotton bundles 5 are clamped between the edge and the plate. The edge shown has two slots 6 in which to 70 run the wall paper cutter Figure 2 and the outer portions of the edge merely serve to hold down the ends of the bundles. These outer portions are unnecessary and in subsequent work were discarded and a simple bar 75 used. 80

The accuracy of the method depends on straightening out the fibers and removing motes and tangles from the bundles. This may be partly done by hand in the ordinary 85 way, but it has been found better to comb the bundles through a stationary comb, in order to more completely remove them and to insure a greater parallelism of fiber. The bundles may also be wet in alcohol and 90 rinsed in water. They are then manipulated between the fingers and become greatly condensed and elongated. When dry they retract, but remain more even and give slightly greater accuracy to the process. 95

It is evident that this ratio of ends to middle is a certain function of the length of the cotton. The longer the cotton the greater the weight of the ends, the middle being constant in length. It is unnecessary however to convert the ratios into lengths as the ratios themselves serve to determine the staple of the cotton and to give its spinning value. 100

However since customs of trade do not as 105 yet recognize these ratios, methods have been devised to convert the ratios into lengths. If the cross sectional area of each fiber were the same from end to end, then it would be possible by this method to develop a formula 110

for the average length of the fiber, however much the different fibers might differ in cross section. It has been found however that cotton fiber has thicker walls and is 5 stronger in the middle than at the ends and presumably it has greater weight per given length at this position. The tip end runs to a point and therefore has less cross section than the seed end. However there is 10 an even possibility of the ends being evenly distributed in the bundle so this factor cancels out.

If the cross section of each fiber were the same from end to end a true average length 15 could be found by the following formula. Let  $L$  be this length and  $M$  the length of the middle portion cut out.  $L-M$  would then be the length of the ends and  $R$  the ratio by weight would equal  $L-M$  divided 20 by  $M$ . Therefore  $L=M(1+R)$  assuming the same density for cellulose in all fibers. Because of the greater thickness of the middle the length found by this formula is something less than the true average length 25 of the fiber. When the middle portion is made one centimeter, then this formula becomes simply  $L=1+R$ .

However no such factor as an average length is now recognized in the trade so 30 work has been done to relate it to the trade lengths. The ratios by weight of the original staple standards preserved by the United States Government were carefully determined. The middle portion was three 35 eights of an inch. The ratios were plotted against the called lengths and the equation of the resulting line determined. These body or trade lengths ran all the way from three quarters of an inch to one and three quarters 40 of an inch, in the main by sixteenth inch jumps. The curve was practically a straight

line, showing the excellence of the work done on the original standards. Substituting the length of the middle in this curve the equation for relating ratios to body lengths 45 became substantially  $L=.7R+2$ , where  $L$  is now the body length.

This process requires but a simple clipping device and a delicate balance. By it the in-expert may surpass the expert in accuracy. 50 The pulls do not require great care in evening up, provided both ends of substantially all fibers are cut at their middle portion. Humidity however before cutting has some effect on the result as it does also in hand 55 stapling.

Having thus described my invention, what I desire to secure by Letters Patent, is:—

1. A method of stapling cotton or other fibers of various lengths, consisting of cutting a fixed length, from substantially all of the fibers at or near their middle portion and determining the ratio by weight of the ends to the middle. 60

2. A method of determining the apparent 65 average length of a number of fibers of varying lengths, consisting of cutting a fixed length from substantially all of the fibers at or near their middle portion, determining the ratio by weight of the ends to the middle 70 and using this ratio in calculating their average length.

3. A method of determining the body or 75 trade length of a number of fibers of varying lengths, consisting of cutting a fixed length from substantially all of the fibers at or near their middle portion, determining the ratio by weight of the ends to the middle portion and the use of this ratio in calculating the trade or body length.

ELBERT E. CHANDLER.